

J. S. GRAVELY,  
SHOT SHELL,  
APPLICATION FILED JUNE 14, 1919.

1,320,754.

Patented Nov. 4, 1919.



Adhesive film comprising polymerized  
Chinese Wood oil.

Inventor.  
Julian S. Gravely  
by Seymour Garce  
Atlys.

# UNITED STATES PATENT OFFICE.

JULIAN S. GRAVELY, OF NEW HAVEN, CONNECTICUT, ASSIGNOR TO WINCHESTER  
REPEATING ARMS CO., OF NEW HAVEN, CONNECTICUT, A CORPORATION.

## SHOT-SHELL.

1,320,754.

Specification of Letters Patent.

Patented Nov. 4, 1919.

Application filed June 14, 1919. Serial No. 304,344.

*To all whom it may concern:*

Be it known that I, JULIAN S. GRAVELY, a citizen of the United States, residing at New Haven, in the county of New Haven and State of Connecticut, have invented a new and useful Improvement in Shot-Shells; and I do hereby declare the following to be a full, clear, and exact description of the same.

10 My invention relates to an improved paper tube for use in the manufacture of paper shot-shells, the object being to produce a smooth, hard and tough tube of superior resistance to moisture, and of a 15 texture which adapts it to hold its crimp. A further object of the invention is to produce such a superior tube without resorting to any operations in addition to those commonly used in the production of paper shot-shell tubes.

With these ends in view, my invention consists in a paper shot-shell tube characterized by a plurality of superimposed coils of paper and co-extensive interposed coils 25 of an adhesive non-hygroscopic film adhering and consolidating the respective coils of paper, the said film containing polymerized Chinese wood oil.

My invention further consists in a paper 30 shot-shell tube having certain details of construction as will be hereinafter described and pointed out in the claims, reference being had to the accompanying drawing, in which the figure is an enlarged view in trans- 35 verse section of a paper shot-shell tube produced in accordance with my invention.

In carrying out my invention, I wind a sheet of suitable paper upon a mandrel after the paper has had applied to one of its faces 40 a continuous film of a paste containing Chinese wood or tung-oil. The moist tube is then dried, preferably in the air, after which it is subjected to heat for a sufficient length of time to polymerize the Chinese 45 wood oil. The tube thus produced consists of a plurality of superimposed coils of paper respectively separated from each other but bound together and consolidated by co-extensive coils of a continuous non-hygro- 50 scopic adhesive film. The polymerization of the Chinese wood oil in the paste makes the tube resistant to moisture, makes it hard and smooth without brittleness, and of a texture which adapts it to hold its crimp. 55 The surface smoothness of the tube is such that it passes through the sizing dies with-

out the employment of the lubricant ordinarily found to be necessary to prevent the exposed fibers of the outer coil of the paper from adhering to the burnished surfaces of the dies. After being sized, the tubes are dipped in a bath of molten paraffin, or a bath consisting of a mixture of paraffin, petrolatum, or other suitable compound for the purpose of impregnating the fibers of the paper so as to render it immune to powder-burns or gas-leaks, as well as to make the tube additionally moisture-resistant, though the primary object of immersing the tubes in a bath of paraffin or equivalent substance, is to treat their interior surfaces in such a manner as to prevent powder-burns and gas-leaks which occur, if at all, from the inside of the tube outward. In this connection it may be said that while the tube is made resistant to moisture by the non-hygroscopic adhesive film coiled between the paper coils, the tube is made proof against powder-burns and gas-leaks by the impregnation of the fibers of the respective coils. I am aware that paraffin as used in the manufacture of paper shot-shell tubes, is ordinarily considered as merely a water-proofing constituent. It is true that paraffin does aid in water-proofing, but paraffin is of even greater importance as used in paper shot-shells in preventing powder-burns which originate solely on the inside of the tube and which are likely to occur if the shells are fired in a hot gun. The fact that paraffin is a great deterrent of powder-burns is more readily demonstrated than explained. It is, however, conceived that it so acts for the reason that being liquefied at the instant of explosion, it envelops the fibers of the paper in a smothering fluid and prevents the access of sufficient oxygen thereto to support combustion.

Paper shot-shells made from such tubes are found to stand up under the endwise thrusts to which they are subjected in the magazine of magazine guns in so far as the paper immediately adjacent to the crimped end of the tube will not upset or swage, nor will the crimp itself open out under the recoil of the arm, whereas tubes as ordinarily made are liable to be upset and uncrimped, due to the fact that the inertia of the load in the shell is markedly greater than the inertia of the paper case. I am aware that it has been proposed to impregnate completed paper shot-shell tubes by

their immersion in solutions containing polymerizable oil, a process less effective and less reliable than my improved method of introducing the polymerizable oil into the 5 paste used to cement the plies of the paper together, for a number of reasons, among which I may mention the certainty I secure of the even distribution of the polymerizable oil throughout the entire structure of the 10 tube due to the fact that the oil is mechanically introduced with certainty and uniformity between the plies of the paper, whereby I eliminate the factors of uncertain distribution due to variations in the absorptive 15 capacity of the paper itself, to variations in the tension under which the tubes are initially wound, and to variations in the moisture-content of the completed tubes when placed in the bath due to variations in the 20 humidity of the atmosphere. Moreover serious objections exist to the use of a bath of polymerizable oil which must be maintained at an elevated temperature to enable it to be driven into the completed 25 tubes. On account of the elevated temperature at which the bath must be maintained, the polymerization of the oil in the bath may take place prior to the introduction of the tubes into it. Thus, if a bath containing 30 polymerizable oil is kept over from day to day at an elevated temperature, it is obvious that a considerable variation in its content of polymerizable oil will result with the effect of making variations in the amount of 35 polymerizable oil actually taken up by the tubes causing the bath-impregnation process to be attended with uncertainty, whereas it is desirable to secure the highest possible uniformity in the amount of polymerizable 40 oil in the tubes. All these objections are overcome by my improved method of introducing the polymerizable oil into the paste the specific character of which may be controlled with more ease and certainty than a 45 bath. Furthermore, a superficially applied coating of polymerizable oil will unavoidably vary in thickness owing to variations in temperature, causing corresponding variations in the viscosity of the bath solution. 50 The above objections apply to processes depending on impregnation in baths. As to all processes of coating paper shot shell tubes with polymerizable oil by spraying or painting, they are open to the objection that 55 they involve a separate group of treatments entailing additional time and labor which must be added to the cost of the tubes. The coating process, moreover, is superficial in character, variable in result, and objectionable in that the coating being superficial rather than integral, may be seriously impaired by abrasion, to that extent reducing the protection aimed at. These results, as

stated, I conceive to be due to the fact that the polymerizable oil when used in the paste 65 is uniformly distributed mechanically throughout the structure of the paper tubes, whereas tubes dependent upon the permeation of the fibers of the paper by waterproofing compounds, vary in density with 70 variations in the compound and the heat under which it is applied, as well as in variations in the density of the paper sheets. My improved shells may be carried in the pocket of a hunter and subjected to long 75 continued abrasion without having their exterior surface abraded or roughened so as to prevent them from functioning in his gun. While I do not limit myself to the employment of any specific paste for the 80 prosecution of my invention, I have secured excellent results by the use of a paste made by boiling starch and water until nearly the required consistency has been secured, and then adding from 4% to 16% of Chinese 85 wood oil and continuing the cooking process with stirring, until thorough emulsification has taken place.

I claim:—

1. As a new article of manufacture, a 90 paper tube for use in the manufacture of paper shot-shells, consisting of a plurality of coils of paper separated by co-extensive interposed coils of a non-hygrosopic adhesive film which binds the coils of the paper together and consolidates them and makes the tube resistant to moisture, the said film containing polymerized Chinese wood oil.

2. As a new article of manufacture, a 100 paper tube for use in the manufacture of paper shot-shells, consisting of a plurality of coils of paper separated by co-extensive interposed coils of a non-hygrosopic adhesive film which binds and consolidates the coils of the paper together, the said film containing polymerized Chinese wood oil and the fibers of the paper being impregnated with a compound resistant to powder-burns.

3. A method of producing paper tubes for use in the manufacture of paper shot-shells, consisting in applying a film of paste containing Chinese wood oil to a sheet of suitable paper, then coiling the paper into a tube, then subjecting the tube to heat for polymerizing the Chinese wood oil contained 115 in the paste, then sizing the tube, and finally subjecting it to a bath of fire-proofing compound for the impregnation of its fibers.

In testimony whereof, I have signed this specification in the presence of two subscribing 120 witnesses.

JULIAN S. GRAVELY.

Witnesses:

DANIEL H. VEADER,  
ERIK S. PALMER.